

# UNITED STATES PATENT OFFICE.

ALEXANDER HILL, OF DUBUQUE, IOWA.

## IMPROVEMENT IN COMPOSITIONS FOR TANNING.

Specification forming part of Letters Patent No. 29,488, dated August 7, 1860.

*To all whom it may concern:*

Be it known that I, ALEXANDER HILL, of Dubuque, in the county of Dubuque and State of Iowa, have invented a new and Improved Composition for Tanning; and I do hereby declare that the following is a full, clear, and exact description of the same.

My invention consists in the employment of a composition of soda, gum-tragacanth, terra-japonica, alum, common salt, saltpeter, and prussiate of potash, mixed together in a certain proportion and dissolved in water, for the purpose of tanning hides and skins.

The proportion in which I mix the above-named ingredients is as follows: soda, one pound; gum-tragacanth, one pound; terra-japonica, twelve pounds; alum, four pounds; common salt, three pounds; saltpeter, one-half pound; prussiate of potash, one-fourth pound. These ingredients are dissolved in water, and the hides or skins, after having been worked in the usual manner, are introduced into this liquor and left there about ten days.

This time is sufficient to finish the tanning process, and the leather produced is superior to other quick-tanned leather. It is not liable to crack, it preserves its toughness, and it resembles in all its properties the leather prepared in the ordinary slow manner. The influence of the soda and tragacanth counteracts the injurious influence of the other ingredients, and these substances prepare the cellules and fibers of the hides or skins to receive and combine with the tanning ingredients.

What I claim as new, and desire to secure by Letters Patent, is—

The employment or use for the purpose of tanning hides or skins of a composition prepared by dissolving in water the above-named ingredients, mixed together in about the proportion herein set forth and described.

ALEXANDER HILL.

Witnesses:

M. H. BEACH,  
GEO. GRAY.